

## UNITED STATES PATENT OFFICE.

NORMAN B. PILLING, OF WILKINSBURG, AND ROBERT E. BEDWORTH, OF PITTSBURGH,  
PENNSYLVANIA, ASSIGNORS TO WESTINGHOUSE ELECTRIC & MANUFACTURING  
COMPANY, A CORPORATION OF PENNSYLVANIA.

## HIGH-TEMPERATURE RESISTOR MATERIAL.

No Drawing.

Application filed October 25, 1921. Serial No. 510,318.

To all whom it may concern:  
Be it known that we, NORMAN B. PILLING, a citizen of the United States, and a resident of Wilkinsburg, in the county of Allegheny and State of Pennsylvania, and ROBERT E. BEDWORTH, a citizen of the United States, and a resident of Pittsburgh, in the county of Allegheny and State of Pennsylvania, have invented a new and useful Improvement in High-Temperature Resistor Material, of which the following is a specification.

This invention relates to resistor material, more particularly to material adapted for use as resistors in furnaces and other heating applications.

Up to the present time, the material in most common use for such applications was an alloy of nickel and chromium which has a high melting point and is well suited for many ordinary heating purposes. However, the alloy, upon exposure to relatively high temperatures, above 1000° C., especially in the presence of air, deteriorates owing to oxidation of the metals of the alloy, and, if the material is in the form of a wire or strip, it is very likely to burn out at the point of high temperature and maximum vaporization.

It is among the objects of our invention to provide a resistor material having the characteristics desirable for heating and similar applications which may be used at relatively high temperatures in an oxidizing or a neutral atmosphere without deterioration.

It is a further object of this invention to provide a material of the character designated which shall be capable of long continued use at a temperature higher than the ordinary operating temperatures of nickel-chromium alloys.

In practising our invention, we provide a non-metallic material, specifically an oxide, having both a low specific resistance and a low negative temperature coefficient of resistivity. Most oxides are either non-conductors or very poor conductors of electricity at ordinary temperatures and, in order to utilize the same for the passage of electric current, it is necessary to first heat the same to a relatively high temperature by external means and allow current to pass therethrough to maintain the temperature

of the oxide. Such an application is made of oxides in the well known Nernst lamp. 55

We have found that cadmium oxide has characteristics widely different from the characteristics of most metal oxides. Whereas most oxides have high negative temperature coefficients, cadmium oxide has a very low negative temperature coefficient. The resistivity of cadmium oxide is approximately .1 ohm per cubic centimeter and is practically constant over a large temperature range, which we have found extends from ordinary room temperatures to 1100° C. and above. The oxide is chemically stable at all temperatures of use, especially at the higher temperatures (500° C. and above) under oxidizing or neutral atmospheric conditions. 65

The material may be formed into any suitable shapes for various purposes. When used as a resistor in heating furnaces, we preferably grind the cadmium oxide to a fine powder, moisten the same with a small amount of water and compress the material into suitable shapes in molds. The molded articles are then heated to a temperature above 800° C., causing sintering and cohesion of the particles resulting in a body which is firmly united into a hard, strong and compact mass, capable of withstanding considerable use and rough handling. 75

As an example of the many uses to which our new material is adapted, we have formed the same into tubes which are adapted to replace the ordinary refractory tube or muffle shape having a coil of wire on the outside thereof for heating purposes. We have also utilized our material in the form of rods and other shapes for heating and for resistors for various purposes. 90

The material has many advantageous characteristics which make it particularly suitable for resistor elements. It has a very low negative temperature coefficient, making it suitable for use at ordinary temperatures as well as at temperatures up to and above 1100° C., and the resistance thereof is low compared to the resistance of other metal oxides. It has a high melting point, a high dissociation temperature and is stable under oxidizing or neutral atmospheric conditions. 100

Although we have described our invention in connection with heating furnaces and

- resistors, it is obvious that the uses of our new material are not limited to those specified but that the range of adaptability thereof includes many other applications.
- 6 In the above description of our invention, we have described the use of cadmium oxide per se, but it is obvious that modifying elements, such as inert diluting materials, conducting materials or high-resistance 10 materials may be added thereto to modify the characteristic and fundamental properties thereof for any special purpose. For example, we have modified cadmium oxide with a small amount of inert refractory 15 material, such as zirconium silicate. This is accomplished by grinding the cadmium oxide with about 5% zirconium silicate to a fine powder, moistening the same with water, compressing and then baking the 20 same to produce a hard, tough, coherent mass.
- We claim as our invention:
1. Resistor material comprising an oxide having a low negative temperature coefficient of resistivity.
  2. Resistor material comprising an oxide having a low negative temperature coefficient of resistivity over a large temperature range.
  3. Resistor material comprising an oxide having a low negative temperature coefficient of resistivity over a temperature range of at least 1000° C.
  4. Resistor material comprising an oxide having a low negative temperature coefficient of resistivity over a temperature range of at least 500° C.
  5. Resistor material comprising an oxide having a low negative temperature coefficient of resistivity over a large temperature range and being chemically stable under oxidizing or neutral atmospheric conditions.
  6. Resistor material comprising an oxide having a low negative temperature coefficient of resistivity over a large temperature range and being chemically stable under ox-

dizing or neutral atmospheric conditions to a temperature of at least 1100° C.

7. Resistor material comprising an oxide having a resistivity of approximately .1 ohm per cc.

8. Resistor material comprising an oxide having a resistivity of approximately .1 ohm per cc. and having a low negative temperature coefficient of resistivity.

9. Resistor material comprising an oxide having a resistivity of approximately .1 ohm per cc. and having a low negative temperature of resistivity over a temperature range of at least 500° C.

10. Resistor material comprising cadmium oxide.

11. Resistor material comprising cadmium oxide and inert refractory material.

12. Resistor material comprising cadmium oxide and a small amount of inert refractory material.

13. Resistor material comprising cadmium oxide and a small amount of zirconium silicate.

14. Resistor material comprising cadmium oxide and approximately 5% of zirconium silicate.

15. A new article of manufacture comprising a compressed, baked mass of cadmium oxide.

16. A new article of manufacture comprising a compressed, baked mass of cadmium oxide and inert refractory material.

17. A new article of manufacture comprising a compressed, baked mass of cadmium oxide and a small amount of inert refractory material.

18. A new article of manufacture comprising a compressed, baked mass of cadmium oxide and a small amount of zirconium silicate.

In testimony whereof, we have hereunto subscribed our names this 18th day of October, 1921.

NORMAN B. PILLING.  
ROBERT E. BEDWORTH.

**Certificate of Correction.**

It is hereby certified that in Letters Patent No. 1,467,810, granted September 11, 1923, upon the application of Norman B. Pilling, of Wilkinsburg, and Robert E. Bedworth, of Pittsburgh, Pennsylvania, for an improvement in "High-Temperature Resistor Materials," an error appears in the printed specification requiring correction as follows: Page 2, line 59, claim 9, before the word "of" insert the word *coefficient*; and that the said Letters Patent should be read with this correction therein that the same may conform to the record of the case in the Patent Office.

Signed and sealed this 23d day of October, A. D., 1923.

[SEAL.]

**WM. A. KINNAN,**  
*Acting Commissioner of Patents.*